

1

2,771,371

## ANTI-RUST OILS

Edgar A. Dieman, Crown Point, and Philip H. Ravenscroft, Munster, Ind., assignors to Standard Oil Company, Chicago, Ill., a corporation of Indiana

No Drawing. Application September 23, 1952,  
Serial No. 311,142

6 Claims. (Cl. 106—14)

This invention relates to improvements in rust preventive compositions and particularly to petroleum base rust preventives for application to metal surfaces in thin, continuous films.

Typical of the coatings applied to metal surfaces for protection from rust are those comprising predominately petroleum products such as lubricating oils, paraffin oils, greases, etc. Rust preventives of this type have given satisfactory protection under some corrosion conditions but not under others. To improve the effectiveness of such compositions, the art suggests that the soaps of preferentially oil soluble sulfonic acid (i. e. mahogany acids) derived from fuming sulfuric acid treatment of petroleum oils be added thereto. U. S. Patents 1,630,101, 1,795,993, and 2,348,715, disclosing broadly the use of soaps of oil soluble sulfonic acids derived from petroleum oils in such compositions, are typical of the art on compositions of that type.

We have now made the surprising discovery that highly effective and very economical rust preventive compositions may be prepared from solvent extracts resulting from the treatment of petroleum oils of lubricating oil viscosity range with solvents such as phenol, Chlorex ( $\beta,\beta'$  dichlorodiethylether), etc. Further, it has been discovered that the effectiveness of such extracts under certain conditions is increased by the addition of mahogany soap or by acid treatment of the extract and that even greater protection is obtainable under some conditions when the extract is both acid treated and admixed with mahogany soap.

Such extracts often, are quite viscous and may require dilution with a suitable hydrocarbon solvent to enable their application in substantially continuous, thin films.

Whether an acid treated or untreated extract should be employed in a given situation and whether a mahogany soap should be added thereto depends to a large extent upon the particular corrosive conditions to which the metal is to be subjected. Thus, in outdoor exposure tests it has been found that although some advantage may be gained by employing an acid treated extract, such is ordinarily insufficient to warrant that additional refinement. Further, the use of mahogany soaps in either acid treated or untreated extract, under the conditions encountered in certain outdoor tests, results in no particular improvement. On the other hand, in humidity cabinet tests the advantage of first acid treating the extract is clearly demonstrated and even greater improvement results from the incorporation of mahogany soaps. The conditions employed and the corrosive atmosphere to which the test plates are subjected in each of these tests are substantially different, as will hereinafter be apparent, and are intended to simulate widely divergent corrosive conditions to which metals may be subjected.

Without being bound by any theory herein expressed or implied, it appears that the oil-solubility and polarity of the particular mahogany soaps employed as well as the polarity of the extracts has a noticeable effect upon

2

properties of the ultimate composition. In general, it has been found that compositions which are either excessively polar or non-polar in character tend to be poorer in rust preventive properties than a more intermediate (with respect to polarity) composition. Thus, for example, although any mahogany soap prepared in accordance herewith may be employed in combination with either treated or untreated extracts to give substantial protection, particular combinations of extracts and mahogany soaps tending to moderate the polarity of the mix have indicated advantages. Thus, the polarity of the soaps, to name only those, in a non-limiting way, which are particularly preferred and in descending order of their polarity, is as follows: sodium AA mahogany soap, sodium B mahogany soap, calcium A mahogany soap, and calcium B mahogany soap. The polarity appears to vary inversely with respect to the molecular weight of the soaps. It has been found, in addition, that acid treated extracts are less polar in nature than those which are untreated. The use of a more polar soap with a treated extract or a less polar soap with an untreated extract, therefore, has given the best results. Unexpected and unexplainable variations in the degree of effectiveness may be encountered, however, and many factors, e. g. the nature of the surface to be protected, the conditions to which it will be exposed, etc. affect the selection of the combination of soap and extract.

The various grades of mahogany acids, from which the soaps referred to above are derived, are produced in a manner well known to the art, i. e. by fuming sulfuric acid treatment of petroleum fractions. The B mahogany acids are produced from the treatment of petroleum oils having a viscosity of from about 100 to about 350 SSU or higher with from about 3 to 6 pounds of fuming acid per gallon of oil. The treated oil is extracted with a 50 to 80% solution of ethyl alcohol in water at about 150° to about 170° F., using a ratio of about one volume of aqueous alcohol for each four volumes of oil. The sulfonic acids may be neutralized before or after extraction from the oil, e. g. by contact with sodium hydroxide solution, and may be purified by further extraction with alcohol to remove salts and water. The mahogany A and AA soaps are prepared in a manner similar to that used for B soaps but employing somewhat lower viscosity oils and lesser amounts of sulfuric acid. The mahogany A soaps are slightly more soluble in water than are the B soaps and the AA grade display even greater water solubility and a definite decrease in oil solubility. Reference is made to U. S. 2,533,700 and U. S. 2,348,715 wherein a more detailed discussion of the nature and preparation of different grades of mahogany acids and soaps is contained. Although described particularly with respect to sodium and calcium soaps other metal soaps, such as are mentioned in the above patents, may be employed herein.

Extracts employed in accordance herewith are those resulting from the solvent treatment of petroleum oils to remove aromatics and other low V. I. compounds. Whereas the extracts of lubricating oils in general have given excellent protection under either outdoor or humidity cabinet tests, it has been found that those compositions derived from the more viscous base oils, particularly SAE 40, furnish the most effective rust preventives in outdoor tests. In general, extracts having a viscosity at 100° F. of from about 500 to 10,000 S. S. U. and preferably from about 3,000 to about 10,000 S. S. U. may be employed. Somewhat higher percentages of an inert organic diluent is preferably employed with the more viscous extracts than is necessary with a less viscous material in order to produce an ultimate rust preventive composition of such viscosity as will enable its being

readily applied to metal surfaces in thin, continuous films. With the less viscous extracts a diluent may be dispensed with if desired.

Solvents employed in the treatment of lubricating oils to remove aromatics and other materials having a low viscosity index are well known to the art; thus, for example, phenol, Chlorex ( $\beta, \beta'$  dichlorodiethylether), furfural, nitrobenzene, sulfur dioxide, and others have been employed for the purpose. The extracts (freed of solvent) obtained by the treatment of lubricating oils with these solvents are of substantially the same type for any given oil and may be employed in accordance herewith. Whereas extracts obtained by extraction of lubricating oils with either Chlorex or phenol are referred to specifically and particularly preferred, extracts resulting from extraction with the other solvents are likewise suitable. Mixtures of such extracts from different sources may also be employed.

The methods by which the above named solvents are employed to treat lubricating oils and the manner in which the extracts are freed of solvent are well-known to the art and it is not intended that such be construed as part of the present invention. Typical examples of such extraction processes are illustrated by U. S. 1,860,823 which describes a phenol extraction process, U. S. 2,003,233 the extraction of a lubricating oil with Chlorex, U. S. 2,161,567 describing extraction with furfural, U. S. 2,251,474 teaching extraction with  $\text{SO}_2$ , etc. Mixtures of such solvents (e. g. U. S. 2,120,810 teaches  $\text{SO}_2$  plus phenol) likewise may be employed.

With respect to the treatment of these solvent extracts with sulfuric acid, it is preferred that the extract itself be acid treated after solvent extraction has occurred. Some of the advantages of an acid treated extract may be obtained, however, when untreated extracts of previously acid treated oils are employed. Sulfuric acid of from about 92% to about 98% strength is preferably employed for the acid treatment of extracts in accordance herewith. About 0.5 pound to 3 pounds of acid per gallon of extract may be employed, preferably from about 1 to 2 pounds per gallon. The acid treatment may take place in the presence of a low boiling solvent such as propane, pentane, etc. Such solvent is removed completely before employing the oil in accordance herewith. Sludge formed is removed by settling before compounding the rust preventive.

Some extracts of the type described are viscous and ordinarily incapable, under normal temperature conditions, of being spread over a metal surface in a relatively thin and continuous film. Accordingly, it is essential to cut their viscosity with a solvent-thinner such as a naphtha, kerosene, benzene, carbon tetrachloride, etc. Stoddard Solvent (sometimes referred to as Cleaner's Solvent) a highly refined naphtha, boiling from about 300° F. to about 400° F., is particularly suitable for the purpose. Petroleum solvents, in general, boiling from about 200° F. to about 450° F. are particularly desirable for the purpose.

In addition to the mahogany soap, solvent extract, and inert organic diluent, the improved rust preventive composition preferably contains a small amount of a compound which comprises a mixture of aliphatic oxygen containing compounds of petroleum origin. These are preferably obtained by controlled oxidation of pure hydrocarbons or mixtures thereof, such as the hydrocarbons occurring in or associated with petroleum oils, in liquid phase at an elevated temperature and under super-atmospheric pressure. These aliphatic compounds contain a mixture of substantial quantities of alcohols, ketones, alcohol-ketones, lactones and esters together with some unoxidized hydrocarbons. The method of obtaining these compounds and the compositions thereof are described in U. S. Patents, 2,090,768, 2,090,769 and 1,863,004 as well as others. Products of this type are

marketed under the trade name of "Alox"; compounds designated as "Alox 350" and "Alox 600" are particularly desirable for this purpose and substantially contribute to the lubricity of the rust preventive compositions as well as, to some extent, enhancing rust preventive properties of the composition. A certain amount of lubricity is desirable in rust preventives employed to coat certain types of metal surfaces. Thus, for example, in steel strapping employed to bind bales of paper, cotton, or boxing of materials, etc., it is necessary that the ends of the strap, which are in contact as the binding is tightened, slide over each other relatively easily with a minimum of friction. The composition of the present invention serves the dual purpose in such cases of preventing rust and lubricating the surfaces.

Rust preventive compositions of the present invention may contain the above described components in the following approximate proportions:

|    |                            | Rust preventive composition <sup>1</sup> |                                  |
|----|----------------------------|------------------------------------------|----------------------------------|
|    |                            | Range (weight percent)                   | Preferred range (weight percent) |
| 20 | Solvent extract            | 70-100                                   | 80-99                            |
| 25 | Mahogany soap <sup>2</sup> | 0-30                                     | 1-5                              |
|    | Alox compound              | 0-10                                     | 1-5                              |

<sup>1</sup> Whereas a diluent is not essential it is ordinarily desirable to employ same in conjunction with such a composition. The diluent should, in any event, comprise not more than about 35% and preferably from about 50 to 75% by weight of a diluted rust preventive composition.

<sup>2</sup> Based upon oil-free soap (petroleum mahogany soaps as recovered by method referred to above ordinarily contain from about 40 to about 70% oil by weight).

<sup>3</sup> "Mahogany Soap" as employed in the above formula and in the appended claims may include only one or a plurality of different grades of preferentially oil-soluble sulfonate, e. g. Sodium B and Calcium A, etc.

The data set forth in Table 1 were obtained in humidity cabinet tests. In such tests, polished or sand blasted cold rolled S. A. E. 1020 steel panels, 2" x 3" x 1/8" were suspended in an atmosphere of 100% humidity at 100° F. in a special cabinet and the time of initial corrosion of the panels is noted. The humidity cabinet is pro-

TABLE 1  
Humidity cabinet test<sup>1</sup>

| 50 | Coating on Panel                                        | Mahogany Soap Employed as Additive |        |        |           |
|----|---------------------------------------------------------|------------------------------------|--------|--------|-----------|
|    |                                                         | None                               | Soda A | Soda B | Calcium A |
|    |                                                         | Hours to Initial Rust              |        |        |           |
| 55 | None                                                    | >8                                 |        |        |           |
|    | Chlorex Extract of SAE 40 Oil                           | >24                                | 135    | 135    | 135       |
|    | Acid Treated Chlorex Extract of SAE 40 Oil              | >24                                | 135    | 279    | 207       |
|    | Chlorex Extract of SAE 20 Oil                           | >24                                | 141    | 480    | 21        |
|    | Acid Treated Chlorex Extract of SAE 20 Oil              | >24                                | 135    | 471    | 207       |
| 60 | Phenol Extract of SAE 10 Oil                            | >24                                | 69     | 165    | 69        |
|    | Acid Treated Phenol Extract of SAE 10 Oil               | >24                                | 189    | 165    | 213       |
|    | Chlorex Extract <sup>2</sup> of Acid Treated SAE 40 Oil | >24                                | 141    | 69     | 717       |
|    | Chlorex Extract <sup>2</sup> of Acid Treated SAE 20 Oil | >24                                | 165    | 189    | 300       |
| 65 | Chlorex Extract <sup>2</sup> of Acid Treated SAE 10 Oil | >24                                | 237    | 333    | 189       |

<sup>1</sup> Test conducted as described above in specification; panels were dipped in composition comprising 63% Stoddard Solvent, 30% extract and 2% sulfonate (oil free basis).

<sup>2</sup> Note that base oil was acid treated prior to extraction.

70 vided with heating units and thermal regulators for automatic temperature control. A water level of about six inches is maintained in the bottom of the cabinet to give approximately 100% humidity at all times. The steel panels are coated by dipping into the rust preventive material, dried overnight, and are suspended by

glass hooks from a revolving stage in the humidity cabinet. From 1 to 1.5 complete changes of saturated air per hour are provided in the cabinet. All extracts employed in tests hereinafter set forth were from dewaxed oils. Those referred to as being acid treated were contacted with one pound of 96%  $H_2SO_4$  per gallon of extract.

As may be observed in Table 1, the compositions of the present invention give substantial protection from corrosion under severe conditions as compared with uncoated panels or extracts without mahogany soaps therein. In general, under the conditions of the tests, the acid treated extract or extract resulting from an acid treated stock provides more protection than a composition derived from an untreated extract. In Table 2 is shown the improvement obtainable by an increase in soap content and the use of a combination of mahogany soaps selected to moderate the polarity of the mixture.

TABLE 2  
Humidity cabinet tests<sup>1</sup>

| Coating on Panels                         | Mahogany Soap Employed as Additive, Wt. (Percent) |           |           | Hours to Failure |
|-------------------------------------------|---------------------------------------------------|-----------|-----------|------------------|
|                                           | Soda AA                                           | Calcium A | Calcium B |                  |
| Phenol Extract of SAE 40 Oil              | 2                                                 | 4         | -----     | 984              |
| Acid Treated Phenol Extract of SAE 40 Oil | 2                                                 | 4         | -----     | 912              |
| Phenol Extract of SAE 40 Oil              | 2                                                 | -----     | 4         | 1,114            |
| Acid Treated Phenol Extract of SAE 40 Oil | 2                                                 | -----     | 4         | 1,013            |

<sup>1</sup> Panels were dipped in composition comprising 70% Stoddard Solvent, 20% extract, 4% calcium soap of "Alox 600" and 6% sulfonate (oil-free basis).

Although the Alox 600 soap employed in the above tests appears to have a beneficial effect upon the rust preventive properties of the composition it is added primarily to impart lubricity to the composition.

In Table 3 are shown the results of outdoor exposure tests in which the effectiveness of untreated extracts is shown to be at least as high (within the limits of observable difference) if not higher than treated extracts. Other outdoor tests in which the time of exposure was somewhat greater (and which are therefore not entirely comparable), indicated that incorporation of mahogany soaps in either treated or untreated extracts resulted in no improvement.

TABLE 3  
Outdoor exposure tests<sup>1</sup>

| Coating <sup>2</sup> on panel                 | Percent of Surface Rusted |
|-----------------------------------------------|---------------------------|
| None                                          | 100                       |
| Phenol Extract of SAE 10 Oil                  | 1                         |
| Acid Treated Phenol Extract of SAE 10 Oil     | 5                         |
| Phenol Extract of SAE 20 Oil                  | 0                         |
| Acid Treated Phenol Extract of SAE 20 Oil     | 5                         |
| Phenol Extract of SAE 40 Oil                  | 0                         |
| Acid Treated Phenol Extract of SAE 40 Oil     | 1                         |
| Chlorex Extract of Acid Treated SAE 10 Oil    | 1                         |
| Chlorex Extract of Acid Treated SAE 20 Oil    | 1                         |
| Chlorex Extract of Acid Treated SAE 40 Oil    | 0                         |
| SAE 10 Oil (raffinate from phenol extraction) | 9                         |
| SAE 20 Oil (raffinate from phenol extraction) | 45                        |
| SAE 40 Oil (raffinate from phenol extraction) | 35                        |

Percentages given in the above specification and the appended claims are on a weight basis unless otherwise specified.

Having thus particularly described our invention, what we claim as novel and desire to protect by Letters Patent is defined by the following claims:

1. The method of treating ferrous metal surfaces which are normally exposed to atmospheric air and moisture to prevent rust formation on said surfaces, which method comprises applying to said ferrous metal surfaces a thin film of a slushing oil consisting essentially of a phenol extract of a petroleum oil of lubricating oil viscosity, from about 1% to about 30% of mahogany soap, and from about 1% to about 10% of a mixture of saturated aliphatic oxygen containing compounds including alkyl esters, lactones, ketones, alcohols, and alcohol ketones, said saturated aliphatic oxygen containing compounds being obtained by partial oxidation of petroleum hydrocarbons.
2. The method of claim 1 wherein said phenol extract has been treated with a sulfuric acid of from about 92% to about 98% strength in an amount of from about 0.5 to about 2.5 pounds of acid per gallon of extract.
3. The method of claim 1 wherein the slushing oil is admixed with from about 1% to 85% of an inert hydrocarbon diluent comprising a petroleum naphtha fraction having a boiling range between about 200° F. and about 450° F. and said diluent is vaporized from the slushing oil film after it is applied to said surfaces so that the extract is the sole hydrocarbon component of the final slushing oil film.
4. A composition for preventing rust formation on ferrous metal surfaces which are normally exposed to atmospheric air and moisture, which composition consists essentially of a phenol extract of a petroleum oil of lubricating oil viscosity, from about 1% to about 30% of mahogany soap, and from about 1% to about 10% of a mixture of saturated aliphatic oxygen containing compounds including alkyl esters, lactones, ketones, alcohols, and alcohol ketones, said saturated aliphatic oxygen containing compounds being obtained by the partial oxidation of petroleum hydrocarbons.
5. The composition of claim 4 in admixture with from about 1% to about 85% of an inert hydrocarbon diluent comprising a petroleum naphtha fraction having a boiling range between about 200° F. and about 450° F.
6. The composition of claim 4 in which said phenol extract has been treated with a sulfuric acid of from about 92% to about 98% strength in an amount of from about 0.5 to about 2.5 pounds of acid per gallon of extract.

References Cited in the file of this patent

UNITED STATES PATENTS

|    |           |                       |               |
|----|-----------|-----------------------|---------------|
| 55 | 2,247,475 | Bray et al. -----     | July 1, 1941  |
|    | 2,279,001 | Matheson et al. ----- | Apr. 7, 1942  |
|    | 2,305,358 | Read -----            | Dec. 15, 1942 |
|    | 2,348,715 | Adams et al. -----    | May 16, 1944  |
|    | 2,383,033 | Wade et al. -----     | May 16, 1944  |

<sup>1</sup> No mahogany soap employed.

<sup>2</sup> SAE 1020 sandblasted panels placed at about a 60° angle and given southern exposure on building roof for 14 days during December and January in Hammond, Indiana; panels were dipped in compositions comprising 1 volume extract and 4 volumes naphtha and dried overnight before beginning test.